

Jan. 19, 1932.

E. F. KERN

1,842,028

METHOD OF RECOVERING LEAD-TIN ALLOYS

Filed Jan. 29, 1929



INVENTOR

Edward Frank Kern  
BY  
Pennie Davis Morris & Edmunds  
ATTORNEYS

## UNITED STATES PATENT OFFICE

EDWARD FRANK KERN, OF NEW YORK, N. Y., ASSIGNOR TO AMERICAN METAL COMPANY, LIMITED, OF NEW YORK, N. Y., A CORPORATION OF NEW YORK

**METHOD OF RECOVERING LEAD-TIN ALLOYS**

Application filed January 29, 1929. Serial No. 335,938.

This invention relates to a method of recovering commercially valuable alloys and metals from complex mixtures of metallic elements, particularly lead-tin alloys. This application is a continuation in part of my co-pending application Serial No. 222,209 filed September 26, 1927.

Large quantities of scrap material containing metals in the form of alloys and mixtures are available. This material is derived from secondary white metal alloys, from the smelting of lead-tin ores and metallurgical by-products and from the refining of lead and tin and of lead-tin alloys. This material, containing alloys of lead and tin, with various impurities including zinc, iron, nickel, antimony, arsenic, bismuth, copper, sulfur, silver and gold is substantially useless because no practicable method of separating the impurities and recovering the lead-tin alloys has been devised heretofore.

It is the primary object of the present invention to recover lead-tin alloys substantially free from impurities and to obtain at the same time the various elements present as impurities in the alloys treated in an economical and commercially feasible manner.

The invention depends upon the discovery that the lead-tin alloys can be separated readily from many of the metals which are mingled in the scrap material by liquation, and that the impure lead-tin alloys thus secured may be separated, provided that the impurities are restricted within certain limits, in a substantially pure condition by electrolyzing under the conditions hereinafter described. The lead-tin alloy is deposited upon the cathode, whereas the impurities are retained in the residue which can be separately treated to recover certain valuable elements therein.

Thus if the raw material includes such elements as zinc, iron, nickel and copper, it is treated preliminarily by liquation at a suitable temperature, so that the lead-tin alloys separate, leaving a residual dross containing most of the impurities. This initial separation should be so conducted as to permit the separation of a lead-tin alloy containing less than 10% of impurities, a result which can

be attained ordinarily by heating the raw material at a temperature of between 300° and 400° C. and withdrawing the metal which is melted at that temperature from the residual dross. If the liquated lead-tin alloy contains more than 10% of impurities, it can be diluted by a suitable proportion of a purer lead-tin alloy to bring the percentage of impurities below the limit mentioned.

The liquated lead-tin alloy may contain a proportion of copper, if copper is present in the raw material. If the copper exceeds 0.5%, it should be removed by heating the lead-tin alloy to about 310° to 315° C. and introducing to the molten alloy about one pound of sulfur per pound of copper to be removed. The dross is skimmed from the metal which is then heated to about 350° C. and cast into anodes.

The residual dross from the initial liquation and any which can be produced in removing copper from the lead-tin alloy are then oxidized and remelted to remove the major portion of the arsenic, sulfur and iron and a part of the antimony which may be present in combinations such as  $Fe_3Sn$ ,  $Fe_2Sn_2$ ,  $Fe_3Sb_2$ ,  $Fe_3As_2$ ,  $Cu_2S$ ,  $Cu_2Sn$ ,  $Cu_3Sb$ ,  $SnSb$ , and  $SnAs$ . After oxidizing and smelting, the material consisting principally of impure lead-tin alloy occluded with the residual dross is mixed with the raw material and again liquated to produce lead-tin alloy containing a lower proportion of impurities suitable for use in preparing the lead-tin anodes which are subsequently electrolyzed to produce substantially pure lead-tin alloy cathode material.

The electrolysis of the lead-tin alloy anodes must be conducted under carefully regulated conditions. As an electrolyte, I prefer to employ solutions containing lead and tin fluosilicates and free fluosilicic acid, lead and tin fluoroborates and free fluoboric acid, or lead and tin cresol sulphonate and free cresol sulphonic acid, or mixtures of such solutions. The electrolyte should include approximately 50 to 125 grams of lead and tin per liter as soluble salts and from 30 to 80 grams per liter of free acid, the specific gravity of the electrolyte ranging from about 1.15 to 1.00

to 1.35. Electrolysis is conducted at a temperature between 40° and 50° C. with electrode current densities of from 10 to 25 amperes per square foot. The lead-tin alloy is dissolved at the anode and deposited at the cathode substantially free from impurities, and the cathode material can be melted and cast into commercial bars.

In order to effect the separation of the lead-tin alloy in a dense mass on the cathode, it has been found desirable to add to the electrolyte an organic reagent such as gelatin or glue or mixtures of either gelatin or glue with cresol. The amount of the organic addition reagent such as gelatin or glue required is about one part by weight to three thousand parts by weight of the electrolyte. The organic addition reagent should be added periodically to the electrolyte as indicated by the characteristic form of the cathode deposit. The organic addition reagents mentioned are merely illustrative, and other reagents adapted to produce the same or similar results with respect to the density of the cathode deposits can be employed.

To ensure continuity and satisfactory operation of the electrolysis, it is essential to circulate the electrolyte from the bath in which electrolysis is conducted to a precipitating tank in which the electrolyte is brought into contact with granulated lead-tin alloy. The circulation should be conducted at the rate of about one gallon per minute per thousand amperes of current flowing. The circulation and the contact with the granulated lead-tin alloy precipitate the impurities which are dissolved in the electrolyte from the anode residues and replaces the lead and tin which are lost as occluded electrolyte in the anode residues and by spillage and leakage of the electrolyte. The concentration of the electrolyte in lead and tin, which is an essential condition for successful operation, is thus maintained substantially constant.

The loss of electrolyte by occlusion in the anode residues and by leakage and spillage averages about 10 pounds per ton of anodes refined for each per cent of impurities that the anodes contain, provided that the anode residues are properly washed and care is taken to prevent excessive losses by spillage and leakage. There is, therefore, a certain loss of acid, and since the concentration of the acid in the electrolyte is an essential condition, it is necessary to add acid from time to time to the electrolyte to make up such losses.

Under the conditions defined and particularly the maintenance of these conditions without substantial variation, it is possible to continuously separate a substantially pure lead-tin alloy at the cathode.

In carrying out the invention there is a portion of anode scrap as well as insoluble

anode residues which accumulate. The scrap is washed to remove the anode residues and to recover the electrolyte. The scrap after washing is remelted into anodes. The residues are filtered and washed to separate the electrolyte which is returned to the circulating tank and mingled with the electrolyte which, after passing over the granulated lead-tin alloy, is returned to the electrolytic bath. The relatively weak wash solutions may be evaporated to a specific gravity of about 1.25 before they are introduced to the electrolyte. The washed anode residues, which will contain antimony, arsenic, bismuth, copper, sulfur, silver and gold if one or more of these metals are present in the lead-tin anodes, may be treated in any desirable way for the recovery of their valuable metal content.

The invention will be more readily understood by reference to the accompanying drawing, which is a flow sheet representing the procedure.

The raw material, consisting of lead-tin alloys from various sources and with impurities such as those hereinbefore mentioned, is liquated in a reverberatory furnace or melting kettle indicated at 5, at a temperature between 300° and 400° C. The molten lead-tin alloy separates and leaves the residual dross. The latter is withdrawn and is oxidized and smelted in a reverberatory furnace indicated at 6. Impurities such as arsenic, sulfur, iron, and antimony are thus removed, and the resulting impure lead-tin alloy indicated at 7 is returned and mixed with the raw material.

If the liquated lead-tin alloy contains more than 10% of impurities, a purer alloy from any suitable source is mixed therewith or the liquation may be repeated in the reverberatory furnace 5 to produce a purer material.

The liquated lead-tin alloy containing less than 10% of impurities is then melted if it contains more than 0.5% of copper in a kettle or furnace indicated at 8, and sufficient sulfur is added when the metal is at a temperature of about 315° C. The sulfur combines with the copper and the resulting dross is skimmed from the metal. It may be mixed with the dross in the furnace 6 and liquated and oxidized therewith. The metal in the kettle or furnace 8 is then heated to about 350° C. and is cast at a temperature between 300° and 350° C. in the form of lead-tin anodes 9 adapted for use in the electrolytic tank 10.

The electrolytic tank is supplied with an electrolyte containing between 50 and 125 grams per liter of lead and tin as soluble salts and from 30 to 80 grams per liter of free acid. The salts and acids used are preferably those hereinbefore mentioned. This electrolyte is circulated constantly between the electrolytic

tank 10 and a precipitating tank 11 which contains a quantity of granulated lead-tin alloy. The circulation is maintained at a rate of about one gallon per minute per 5 thousand amperes used.

Electrolysis is conducted in the electrolytic tank 10 at a temperature of about 40° to 50° C. with electrode current densities between 10 and 25 amperes per square foot, 10 the circulation being meanwhile maintained continuously. Fresh anodes are supplied as they are consumed, and the cathodes consisting of the pure lead-tin alloy are removed from time to time.

15 A proportion of organic addition reagent equal to one to two pounds per ton of anodes treated or about one part by weight to three thousand parts by weight of the electrolyte is added gradually to the electrolyte, the addition being governed by the appearance of the cathodes. Similarly sufficient acid is added from time to time to replace that lost in the anode residue and by leakage and spillage.

25 The pure lead-tin cathodes removed from the bath are melted in a furnace 12 and cast into commercial bars. The lead-tin alloy thus recovered is suitable for numerous commercial uses, being substantially free from 30 impurities which would seriously affect the quality of the metal.

The anode scrap and the anode residues are removed from the electrolyte and washed at 35 13. The anode scrap is then remelted at 14 and returned in the form of fresh anodes to the electrolyte. The anode residues are filtered and washed at 15, the electrolyte recovered being returned directly to the tank 11. The weak wash solutions are evaporated 40 at 16 and the concentrated solution is then delivered to the tank 11.

The operation as described involves the substantially complete utilization of the raw material and the recovery therefrom in particular of commercial lead-tin alloys constituting the most valuable portion of the raw scrap material. The operation is readily controlled and can be carried out economically and efficiently. The method affords, therefore, a practicable procedure 45 whereby scrap material is converted into valuable commercial products.

Various changes may be made in the details of the method as described especially to 55 accommodate the operation of the differing compositions of the raw materials treated without departing from the invention or sacrificing the advantages thereof.

I claim:

60 1. The method of recovering lead-tin alloys which comprises electrolyzing anodes consisting of impure alloys of lead and tin in a bath containing from 50 to 125 grams of soluble salts of lead and tin and from 30 to 65 80 grams of free acid per liter of electrolyte.

2. The method of recovering lead-tin alloys which comprises electrolyzing anodes of lead and tin containing not more than 10% of impurities in a bath containing from 50 to 125 grams of soluble salts of lead and tin and from 30 to 80 grams of free acid per liter of electrolyte. 70

3. The method of recovering lead-tin alloys which comprises electrolyzing anodes consisting of impure alloys of lead and tin in a bath containing from 50 to 125 grams of soluble salts of lead and tin and from 30 to 80 grams of free acid per liter of electrolyte, and continuously circulating the electrolyte between the electrolytic bath and a body of lead-tin alloy to precipitate dissolved impurities and to maintain the concentration of lead and tin therein. 80

4. The method of recovering lead-tin alloys which comprises electrolyzing anodes of lead and tin containing not more than 10% of impurities in a bath containing from 50 to 125 grams of soluble salts of lead and tin and from 30 to 80 grams of free acid per liter of electrolyte and continuously circulating the electrolyte between the electrolytic bath and a body of lead-tin alloy to precipitate dissolved impurities and to maintain the concentration of lead and tin therein. 90

5. The method of recovering lead-tin alloys from scrap material which comprises liquating the material to separate impure lead-tin alloy therefrom, adding lead-tin alloy containing a low proportion of impurities to reduce the total impurities below 10%, and electrolyzing anodes of such alloy in a bath containing from 50 to 125 grams of soluble salts of lead and tin and from 30 to 80 grams of free acid per liter of electrolyte. 95

6. The method of recovering lead-tin alloys from scrap material which comprises liquating the material to separate impure lead-tin alloy therefrom, adding sulfur to the molten alloy to remove copper therefrom, and electrolyzing anodes of such alloy in a bath containing from 50 to 125 grams of soluble salts of lead and tin and from 30 to 80 grams of free acid per liter of electrolyte. 105

7. The method of recovering lead-tin alloys from scrap material which comprises liquating the material to separate impure lead-tin alloy therefrom, electrolyzing anodes of such alloy containing not more than ten per cent of impurities in a bath containing from 50 to 125 grams of soluble salts of lead and tin and from 30 to 80 grams of free acid per liter of electrolyte, and continuously circulating the electrolyte between the electrolytic bath and a body of lead-tin alloy to precipitate dissolved impurities and to maintain the concentration of lead and tin therein. 115

8. The method of recovering lead-tin alloys from scrap material which comprises liquating the material to separate impure lead-tin alloy therefrom and electrolyzing anodes 130

of such alloy in a bath containing from 50 to 125 grams of soluble salts of lead and tin and from 30 to 80 grams of free acid per liter of electrolyte.

9. The method of recovering lead-tin alloys from scrap material which comprises liquating the material to separate impure lead-tin alloy therefrom, adding lead-tin alloy containing a low proportion of impurities to reduce the total impurities below 10%, and electrolyzing anodes of such alloy in a bath containing from 50 to 125 grams of soluble salts of lead and tin and from 30 to 80 grams of free acid per liter of electrolyte.

10. The method of recovering lead-tin alloys from scrap material which comprises liquating the material to separate impure lead-tin alloy therefrom, electrolyzing anodes of such alloy in a bath containing from 50 to 125 grams of soluble salts of lead and tin and from 30 to 80 grams of free acid per liter of electrolyte, and continuously circulating the electrolyte between the electrolytic bath and a body of lead-tin alloy to precipitate dissolved impurities and to maintain the concentration of lead and tin therein.

11. The method of recovering lead-tin alloys from scrap material which comprises liquating the material to separate impure lead-tin alloy therefrom and electrolyzing anodes of such alloy containing not more than 10% of impurities in a bath containing from 50 to 125 grams of soluble salts of lead and tin and from 30 to 80 grams of free acid per liter of electrolyte.

In testimony whereof I affix my signature.  
EDWARD FRANK KERN.